

## UNITED STATES PATENT OFFICE

2,286,198

ALLOY WROUGHT IRON AND ARTICLE MADE  
THEREFROMJohn W. Davis, Tarentum, Pa., and Ray McBriar,  
Denver, Colo.No Drawing. Application September 19, 1940,  
Serial No. 357,440

4 Claims. (Cl. 75—123)

Our invention relates to alloy wrought iron and articles made therefrom such as stay-bolts which have to maintain a high degree of strength up to temperatures in the neighborhood of around 900° F. and which, when in use, are subjected to vibratory stresses, engine bolts which, when in use, are subjected to vibratory stresses and in some instances to approximately the same temperatures, and other articles which have to maintain a high degree of strength under vibratory stresses and relatively high temperatures.

Stay-bolts, engine bolts and many other articles are still manufactured from wrought iron of the types known as refined bar iron and "double refined" iron, even though the cost of such wrought irons is in excess of many of the modern alloy steels.

Wrought iron of the grades now used in the manufacture of these articles has a tensile strength, lbs. per sq. in. (p. s. i.) of from about 47,000 to 52,000 at room temperatures and around 70,000 at about 400° F. Above 400° F., the tensile strength drops fairly rapidly, for example, at about 750° F., it is from about 32,000 to about 33,000 lbs. per sq. in. and at about 900° F. from about 18,000 to about 20,000.

Stay-bolts not only require high tensile strength at room temperatures, but since they are used in modern locomotives they require high tensile strength at elevated temperatures as well. Stay-bolts, as well as engine bolts, not only require high tensile strength, but must be capable of withstanding vibratory stresses over long periods and must also be readily machineable.

An object of this invention is to produce an alloy wrought iron for use in the manufacture of stay-bolts, engine bolts and other articles having a materially increased tensile strength at room temperatures and at temperatures ranging up to about 900° F. over the same articles made from typical "double refined" wrought iron.

Another object is to produce articles such as stay-bolts and engine bolts from an alloy wrought iron containing from about .10% to about 1.00% of molybdenum and having a yield point p. s. i. at about 900° F. of from about 5,000 to about 8,000 greater than similar articles made from typical "double refined" wrought iron.

An object of this invention is to produce wrought iron containing molybdenum in appreciable amounts up to about 1.00 and which is characterized by a tensile strength when at 750° F., of from 5000 to 6000 lbs. per sq. in. greater than typical wrought iron.

A further object is to produce wrought iron

having a yield point p. s. i. at 750° F. of from about 4000 to about 6000 greater than typical "double refined" wrought iron.

A still further object is to produce an alloy wrought iron having a yield point p. s. i. at 900 F. of from about 5000 to about 8000 greater than typical "double refined" wrought iron.

The molybdenum content of our alloy wrought iron may vary from about .10% to about 1.00% but we prefer to keep it from about .25% to about .50% since "double refined" iron containing molybdenum within this range, is highly satisfactory as to cost, tensile strength and its ability to withstand vibratory stresses.

In comparative vibratory tests made on bars of "double refined" wrought iron having a molybdenum content of from about .39% to about .43% and bars of the same type of wrought iron but without molybdenum, the bars containing molybdenum withstood an average of 272,000 vibrations as against an average of 109,800 vibrations for the bars containing no molybdenum.

We prefer to manufacture our alloy wrought iron by the hand puddling process, and in such process, we prefer to use what is known as the "roasting" method as distinguished from the "scaling" method, although we have obtained quite satisfactory results with the "scaling" method.

In the "roasting" method, after charging the pig iron, the furnace is closed, and by hand firing for a period of from 40-50 minutes the pig iron becomes a molten mass which is then permitted to "roast" for a period of from 20-25 minutes.

Roasting is simply a firing operation with the damper of the furnace up or "flying," during which period some carbon, phosphorus and sulphur are removed. We have found that satisfactory results are obtained by adding to the molten iron immediately before beginning the roasting period, a sufficient quantity of molybdenum to obtain the molybdenum content desired in the finished iron.

We have obtained satisfactory results by using molybdenum tri-oxide, such as sold by the Climax Molybdenum Company under the name of "Molybdic oxide briquettes" and which have the following composition:

|                      | Per cent |
|----------------------|----------|
| Molybdenum tri-oxide | 70-75    |
| Carbon, max.         | 12.0     |
| Iron, max.           | 3.0      |
| Sulphur, max.        | 0.25     |
| Insoluble residue    | 10.30    |

The briquettes melt during the 20-25 minute roasting period and we have found that the metallic molybdenum reduced from the molybdenum tri-oxide is distributed evenly throughout the entire metal mass.

When the "scaling" method is employed, we have obtained satisfactory results by placing the molybdc oxide briquettes on top of the pig iron immediately after the pig iron has been charged in the furnace; both the pig iron and the briquettes being melted in the first operation. No molybdenum apparently is lost during boiling which takes place when the mill scale is added after the melt.

We make use of no special slag but prefer a slag having approximately the following composition:

|                      | Per cent |    |
|----------------------|----------|----|
| Silica               | 16-20    |    |
| Alumina              | 4-6      | 20 |
| Manganese dioxide    | 3        |    |
| Phosphorus pentoxide | 1        |    |
| Ferric oxide         | 70-76    |    |

The molybdc oxide briquettes cause no carbon pick-up since the entire carbon content thereof is utilized in reducing the molybdenum tri-oxide through several stages to metallic molybdenum; all of the carbon being converted into carbon dioxide ( $CO_2$ ) which passes off as gas.

The following data was derived from tests carried out on six bars of our alloy wrought iron, the analyses of which read as follows:

|    | Per cent  |    |
|----|-----------|----|
| C  | .013-.04  | 35 |
| Mn | .05-.06   |    |
| P  | .102-.127 |    |
| S  | .009-.014 |    |
| Si | .099-.141 |    |
| Cu | .040-.050 | 40 |
| Mo | .39-.48   |    |

|                            | 1      | 2      | 3      | 4      | 5      | 6      |
|----------------------------|--------|--------|--------|--------|--------|--------|
| <i>Room temperature</i>    |        |        |        |        |        |        |
| B. H. N.                   | 100    | 100    | 101    | 101    | 100    | 101    |
| Yield point, p. s. i.      | 34,700 | 37,100 | 36,600 | 39,600 | 36,300 | 38,000 |
| Tensile strength, p. s. i. | 52,200 | 52,100 | 52,200 | 52,200 | 52,000 | 52,800 |
| Elong., percent            | 30     | 32.5   | 31     | 31     | 34     | 33     |
| R. A., percent             | 49.0   | 50.0   | 49.0   | 51.0   | 50.0   | 52.5   |
| <i>400° F.</i>             |        |        |        |        |        |        |
| Yield point, p. s. i.      | 31,100 | 30,800 | 31,400 | 30,500 | 31,900 | 33,000 |
| Tensile strength, p. s. i. | 72,000 | 68,700 | 73,000 | 72,400 | 74,000 | 71,500 |
| Elong., percent            | 21     | 20     | 20     | 21     | 20     | 20.0   |
| R. A., percent             | 34.5   | 35.0   | 34.5   | 36.5   | 37.0   | 36.0   |
| <i>750° F.</i>             |        |        |        |        |        |        |
| Yield point, p. s. i.      | 27,600 | 27,450 | 26,050 | 26,250 | 27,300 | 27,440 |
| Tensile strength, p. s. i. | 58,500 | 57,200 | 56,000 | 56,400 | 57,600 | 57,600 |
| Elong., percent            | 25     | 24     | 26     | 24     | 26     | 25     |
| R. A., percent             | 49.0   | 47.5   | 50.5   | 51.0   | 49.0   | 48.5   |
| <i>900° F.</i>             |        |        |        |        |        |        |
| Yield point, p. s. i.      | 25,100 | 24,800 | 24,600 | 24,090 | 28,650 | 26,200 |
| Tensile strength, p. s. i. | 43,000 | 43,500 | 43,500 | 43,200 | 41,700 | 44,300 |
| Elong., percent            | 24     | 24     | 24     | 25     | 25     | 24     |
| R. A., percent             | 53.0   | 53.0   | 53.5   | 54.4   | 55.0   | 54.4   |

In making the above tests, A. S. T. M. standard 2" gauge length test specimens were machined from different bars. Duplicate tension tests were run on bars of each identification number at room temperature, at 400° F., at 750° F. and at 900° F.

The bars were set up in special holders in a hydraulic tension testing machine. A resistance wound cylindrical type electric furnace, split through the axis and mounted with its axis in vertical direction, was used to heat the specimens

and maintain them at the desired temperature during the quick tensile test.

The temperature of the furnace was automatically controlled to within + or - 5° F. of the specified temperature. Two thermocouples were used to determine the temperature of the test specimen. One of these thermocouples was at one end of the gage length and one at the other. The temperature differential between these two thermocouples never exceeded 5° F. throughout any of the tests.

The tension specimens were brought up to the desired temperature and held at that temperature thirty minutes before any load was applied. During the test the cross-head speed of the machine was controlled at .05 to .06" per minute.

Yield points were determined from the plots as recorded by the automatic autographic indicator of the Tinius-Olsen testing machine.

We have found that the addition of from .20 to .50% molybdenum increases the tensile strength of wrought iron at room temperatures by from 1500 to 2000 pounds per square inch, and that when subjected to the higher temperatures of modern locomotive fire boxes, stay-bolts made from our alloy wrought iron have a tensile strength of from 5000 to 6000 pounds per square inch greater than stay-bolts made from typical "double refined" wrought iron.

We have also found that the addition of molybdenum within the range used by us results in a finer and more homogeneous grain structure. This is of distinct advantage, since a large percentage of the stay-bolts are furnished with either a  $\frac{1}{16}$ " or  $\frac{3}{32}$ " diameter hole drilled partially or throughout their entire length. These are then threaded either partially or throughout their entire length.

We have found that articles such as stay-bolts and engine bolts made from hot rolled material embodying our invention are much freer from

scale and have fewer surface pits and other surface defects than similar articles made from hot rolled typical "double refined" wrought iron.

We believe that both stay-bolts and engine bolts made from our alloy wrought iron will have an increased service life of from two to four years longer than the service life of stay-bolts and engine bolts made from typical "double refined" wrought iron. The method of making alloy wrought iron disclosed but not claimed herein constitutes the subject matter of a copending

divisional application for patent filed by us on April 4, 1942, and serially numbered 437,684.

Having thus described our invention, what we claim as new and desire to secure by Letters Patent is:

1. An alloy wrought iron aggregated from a solidifying mass of pasty particles of highly refined metallic iron alloyed with molybdenum, with which, without subsequent fusion, is intentionally incorporated a substantially uniformly distributed quantity of slag in an amount such as is normally present in wrought iron; said alloy containing from about .10% to about 1.00% molybdenum, carbon less than about .06%, with the balance substantially all iron except for said slag and the usual impurities present in wrought iron.

2. An alloy wrought iron aggregated from a solidifying mass of pasty particles of highly refined metallic iron alloyed with molybdenum, with which, without subsequent fusion, is intentionally incorporated a substantially uniformly distributed quantity of slag in an amount such as is normally present in wrought iron; said alloy containing from about .20% to about .50% molybdenum, carbon less than about .05%, manganese not over .06%, with the balance substantially all iron except for said slag and the usual impurities present in wrought iron.

3. An article which, during use, is subjected to relatively high temperatures and vibratory stresses; said article being fabricated from an alloy wrought iron aggregated from a solidifying mass of pasty particles of highly refined metallic iron alloyed with molybdenum, with which, without subsequent fusion, is intentionally incorporated a substantially uniformly distributed quantity of slag in an amount such as is normally present in wrought iron; said alloy containing from about .10% to about 1.00% molybdenum, carbon less than about .06%, with the balance substantially all iron except for said slag and the usual impurities present in wrought iron.

4. A bolt fabricated from an alloy wrought iron aggregated from a solidifying mass of pasty particles of highly refined metallic iron alloyed with molybdenum, with which, without subsequent fusion, is intentionally incorporated a substantially uniformly distributed quantity of slag in an amount such as is normally present in wrought iron; said alloy containing from about .20% to about .50% molybdenum, carbon less than about .05%, manganese not over .06%, with the balance substantially all iron except for said slag and the usual impurities present in wrought iron.

JOHN W. DAVIS.  
RAY MCBRIAN.